

## UNITED STATES PATENT OFFICE.

DAVID J. GILES, OF LATROBE, PENNSYLVANIA, ASSIGNOR TO LATROBE ELECTRIC STEEL COMPANY, OF LATROBE, PENNSYLVANIA, A CORPORATION OF PENNSYLVANIA.

## STEEL ALLOY.

No Drawing.

Application filed April 2, 1926. Serial No. 99,380.

The invention relates to that class of alloy steels, ordinarily known as stainless, which are resistant to attacks of such acids and other substances as are met with in the customary uses of the steels. As heretofore produced, such steels, while having fairly good stainless properties when hardened and polished, have poor stainless properties in their unannealed soft state, and even when heat-treated to bring out their best physical properties they are only fairly strong and ductile.

The object of the invention is to provide a steel alloy of this type which is highly resistant to attack in its annealed as well as in its hardened state, and which in its heat-treated condition is very strong and ductile.

The alloy steel provided according to the invention contains from about .50 to .80% carbon and from about 16.00 to 19.00% chromium, the remainder being iron except for the usual amounts of other elements such as sulphur, phosphorus, silicon and manganese, which are ordinarily present as impurities or as incidental to manufacturing processes. The sulphur and phosphorus should be as low as possible, while silicon and manganese may be present to the extent of about .50% of each, as in most steels. Within this relatively small range of carbon and chromium content the preferred steel alloy contains about .60% carbon and about 17.00% chromium.

As an example of the stainless property of the preferred analysis of this steel in its annealed state, samples of it having a Brinell hardness of 170, when subjected to the standard copper sulphate test showed a deposit of but .00246 grams of copper, when subjected to the standard nitric acid test they showed that no metal was removed, and when subjected to the standard acetic acid test they showed a removal of but .0070 grams of metal. In its hardened state samples of the same steel alloy having a Brinell hardness of 555, when subjected to the standard copper sulphate test showed a deposit of but .00082

grams of copper, and when subjected to the standard nitric acid and acetic acid tests they showed a removal of no metal.

As to the physical properties of the preferred analysis of this steel alloy, annealed samples having a Brinell hardness of 187 showed an average elastic limit of 74540 lbs. per square inch, a tensile strength of 101180 lbs. per square inch, an elongation of 23% in two inches, and a reduction of area of 54.3%. In a semi-annealed state, having a Brinell hardness of 217, samples of the same steel alloy showed an average elastic limit of 84080 lbs. per square inch, a tensile strength of 106530 lbs. per square inch, an elongation of 22% in two inches, and a reduction of area of 50.4%. In a heat-treated hardened state, having a Brinell hardness of 269, samples of the same steel showed an average elastic limit of 121770 lbs. per square inch, a tensile strength of 134500 lbs. per square inch, an elongation of 13% in two inches, and a reduction of area of 39.8%.

From the foregoing it abundantly appears that the improved stainless steel alloy is highly resistant to attack in its annealed as well as in its hardened state, and that it has great strength and ductility. These properties, both stainless and physical, are much superior to those of any known stainless steel on the market. In addition to this, the improved steel has a higher degree of hardening, retains a better cutting edge, and is easier and cheaper to manufacture than any known stainless steel on the market.

I claim as my invention:

A steel alloy consisting of about .60% carbon, and about 17.00% chromium, the remainder being iron except for the usual amounts of other elements present as impurities and as incidental to manufacturing processes, the alloy being highly resistant to attack in its annealed as well as in its hardened state.

In testimony whereof, I sign my name.

DAVID J. GILES.